

July 12, 1927.

1,635,829

O. A. FREDERICKSON

PROTECTING COATING FOR COVERED CONDUCTORS AND METHOD OF APPLYING THE SAME

Filed March 22, 1927

2 Sheets-Sheet 1

*Fig. 1*



*Fig. 2*



*Fig. 3*



*Fig. 7*



*Fig. 8*



INVENTOR:

Otto A. Frederickson

BY *John O. Haas*

ATTORNEY

July 12, 1927.

O. A. FREDERICKSON

1,635,829

PROTECTING COATING FOR COVERED CONDUCTORS AND METHOD OF APPLYING THE SAME

Filed March 22, 1927

2 Sheets-Sheet 2

*FIG. 4*



*FIG. 5*



*FIG. 6*



INVENTOR:

Otto A. Frederickson  
BY *Bob O'Hanis*.

ATTORNEY

Patented July 12, 1927.

1,635,829

# UNITED STATES PATENT OFFICE.

OTTO A. FREDERICKSON, OF WETHERSFIELD, CONNECTICUT, ASSIGNOR TO THE WIRE-MOLD COMPANY, OF HARTFORD, CONNECTICUT, A CORPORATION OF CONNECTICUT.

PROTECTING COATING FOR COVERED CONDUCTORS AND METHOD OF APPLYING THE SAME.

Application filed March 22, 1927. Serial No. 177,424.

This invention relates to a novel protecting coating for the outer jacket of insulated electrical conductors and flexible conduits, and also to a method of applying such coating. The present application is filed as a continuation in part of the Frederickson application Serial No. 144,379, filed October 26, 1926.

Insulated electrical conductors and cables are usually provided with one or more protecting layers or coverings formed of fibrous substances, such as cotton or other inflammable material, and when these conductors are installed in buildings it is important that they be enclosed in metal conduits or be otherwise protected to reduce the fire hazard.

It has therefore been proposed heretofore to apply a coating of flame-retarding compound such as stearin pitch or other suitable fatty acid pitches to the outer surface of such covering of insulated electrical conductors to increase their flame-retarding properties, but these flame-retarding compounds impart to the covering a sticky outer surface that causes the adjacent coils of the covering to stick together when the cable is wound into coils ready for the market. This tendency of the coils to stick together, not only makes the cable hard to uncoil, but is further objectionable since when the stuck coils are forced apart portions of the flame-retarding coating are frequently torn from the cable covering.

To overcome this difficulty it is now the usual practice to apply powdered mica to the flame-retarding coating of the conductor or cable covering, and while the mica reduces the tendency of the adjacent coils to stick together, it does not entirely correct this difficulty, and is objectionable, because it flakes off readily, thus exposing the sticky coating, and furthermore the loose detached flakes of mica become scattered over the floor of the building and other objects during installation of the cable. Such treated conductor coverings are open to a further objection in that the sticky nature of the flame-retarding coating makes the cable difficult to draw through conduits, partitions and floors and around corners during installation. If a covered conductor is subjected to a severe pulling strain during installation the conductor may be stretched or drawn

out by the pulling force until the diameter of the conductor wire is reduced to such an extent that it will heat up when carrying the electrical load for which it was designed, thus increasing the danger of fire, and moreover such pulling strain may cause the covering itself to be injured.

Having the foregoing in mind the present invention relates to a protecting flexible coating for the outer jacket of electrical conductors and conduits, and to a method of applying the coating, whereby the outer surface of the jacket is given the desired flame-repelling properties and at the same time is rendered smooth and clean, to the end that the adjacent coils will not stick together, or the conductor or its covering be injured during installation.

In carrying out the present invention the fibrous covering of an insulated conductor or conduit is given a coating of a flame-retarding compound and over this coating is applied a film of wax-like material such as paraffin, the latter being so applied that there is substantially no mixture of the wax-like material with the flame-retarding compound. As a result of the application of the wax-like material to the sticky flame-retarding compound, a smooth, clean, non-sticky outer surface is imparted to the covering of the insulated conductor or conduit, while the flame-retarding properties of the protecting coating are not appreciably decreased by the presence of the wax-like material. This is due to the fact that the wax material is applied to the coated conductor covering in a thin layer such that there is not sufficient wax material present upon the flame-retarding coating to support combustion, and also to the fact that the wax-material is not mechanically mixed with the flame-retarding material but is applied over the flame-retarding coating to which it adheres.

The application of wax-like material to insulated electric conductors for the purpose of rendering such conductors waterproof is not new and it has been proposed heretofore to immerse insulated conductors in a bath of melted wax or paraffin to cause saturation of the insulation and thereby exclude moisture from the interior of the insulating material, but the application of a wax-like material as a film over a sticky

or adhesive flame-retarding coating previously applied to the insulating fibrous covering or conduit to impart a smooth, non-sticky exterior surface that is flame repellent in accordance with the present invention is believed to be broadly new.

The features of the present invention and new method will be best understood from the following description when read in connection with the accompanying drawings, wherein:

Fig. 1 is a perspective view of an electrical cable the outer jacket of which is provided with the protecting coating forming the subject matter of the present invention;

Fig. 2 on an enlarged scale is a transverse sectional view through the cable of Fig. 1;

Fig. 3 is a perspective view of a conduit for electrical conductors and is shown as provided with the protecting coating of the present invention;

Fig. 4 is a vertical sectional view through mechanism for saturating the outer covering of an insulated conductor with a moisture proofing liquid;

Fig. 5 is a vertical sectional view through somewhat similar mechanism for applying a flame-retarding coating to the cable that has been rendered moisture proof by the treatment of Fig. 4;

Fig. 6 is a vertical sectional view through mechanism for applying a thin coating of wax material to the cable that has been flame-proofed by the treatment of Fig. 5;

Fig. 7 is a diagrammatic view of means for winding a treated insulated conductor into coils ready for the market; and

Fig. 8 is a perspective view of a shipping container for a coiled cable.

The protecting coating forming the subject matter of the present invention may be applied to the outer jacket of an insulated conductor, or it may be applied to a flexible tube for a conductor or to a cable formed of two or more covered conductors, or it may be employed for still other purposes, but in the present instance of the invention it is shown and will be described as applied to the outer fibrous jacket or covering of an electrical cable.

The insulated electrical cable illustrated in the drawings is shown as provided with two metallic conductors 10, each of which has an insulating jacket 11 formed of rubber, and about this jacket is placed a covering 12 of fibrous material. Around the covering 12 of each conductor is placed a further insulating cover 13 and the two insulated conductors thus formed are enclosed in an outer jacket 14 of fibrous material. The valleys formed between the insulated conductors have the fillers 15 laid therein to fill up the air space between the conductors and outer jacket.

The particular construction of the cable so far described forms no essential part of the present invention but is illustrated as showing a type of non-metallic sheathed cable that has received the approval of the Underwriters' Laboratories. The outer covering or jacket upon which the coating forming the subject matter of the present invention is applied, may be braided, woven or otherwise constructed.

The conduit illustrated in Fig. 3 is shown as a woven tube constructed of the longitudinally extending warp threads 16 and the spirally disposed weft threads 17, the warp threads may be formed of thick stiff paper while the weft threads 16 are formed of cotton. However, the particular construction of the conduit forms no essential part of this invention.

While the protecting coating of the present invention is described herein as applied to the outer jacket 14 of the cable it will be understood that such coating may be applied to the conduit of Fig. 3, to a single insulated conductor such as the jacket 12 of the conductor 10, or to various other forms of insulated cables or conductors.

In carrying out the present invention the covered electrical conductor or the conduit is preferably first subjected to a moisture proofing treatment to render the covering or jacket of the conductor or conduit water-proof. This may be done by drawing the covered conductor or conduit from a supply reel 18 (see Fig. 4) over a roll 19, and into a tank 20 containing the moisture proofing substance 21 which may be bituminous material, such, for instance, as asphalt, pitch, or the like. This substance should have high penetrating properties that will penetrate into the centre of the strands forming the covering or jacket 14, and is preferably applied at a high temperature to cause it to drive out the moisture present in the conductor covering. The tank 20 may be heated by a gas burner 22, and as the treated covered conductor leaves the tank the excess liquid is removed therefrom.

This may be done by passing the covered conductor or jacket through a die 24 which may be formed of metal and the bore of which is preferably slightly smaller than the conductor covering so that the die will act to squeeze from the conductor covering the excess liquid. This is important for if an excess amount of the moisture proofing substance is allowed to remain in the cable it will decrease the effectiveness of the flame-retarding coating to be subsequently applied. The treated covered conductor or conduit upon leaving the die 24 is passed several times around the upper drum 25 and lower drum 26 to cool the same and is then wound upon the take-up reel 27 ready for the flame-repellent treatment.

This second treatment may be conveniently effected by the mechanism shown in Fig. 5 wherein the moisture proofed covered conductor in the present instance of the invention is led from the reel 28 over a roll 29 into a heated tank 30 containing a flame-retarding compound 31 such as stearin pitch or other suitable fatty acid pitch later described that is heated by the burner 22. The flame-retarding compound has less saturating properties than the moisture proofing material 21 and consequently forms a coating upon the covering of the conductor or the conduit over the moisture proofing material, the latter serving as a binder that helps to secure the flame-retarding coating to the covering or conduit.

The thickness of the coating 31 upon the jacket 14 is controlled in the present instance by the size of the die 32 formed of metal or other hard material and through which the cable passes as it leaves the tank 30. This die is given a bore that is slightly larger than the cable passing therethrough, so that a layer or coating of the fire-retarding compound which is just thick enough to completely cover and protect the surface of the covered conductor or the conduit is permitted to remain thereon. Other means than the die 32 may be employed to determine the thickness of this coating, but the use of a die serves to accurately control the thickness of the coating and also to smooth or iron the coating material so that it will completely cover the conductor jacket.

As stated the flame-retarding compound is sticky or adhesive, which makes the treated covered conductor difficult to handle; it may therefore be guided from the die 32 through a receptacle 33 containing powdered mica. This mica treatment is employed merely for the purpose of reducing the sticky condition of the cable covering during its manufacture, and is not an essential feature of the finished product.

It is important that the hot flame-retarding compound 31 applied to the textile covering or conduit be cooled prior to the wax or paraffine treatment so that the subsequent application of the wax or paraffine will not cause the same to mix with the flame-retarding compound, because such mixture would impair the fire-repellent properties of the flame-retarding compound.

Stearin pitch is an excellent flame-retarding compound due to its high melting point that ranges from about 250° to 275° Fahrenheit, and also due to its properties of expansion under the application of heat so that it forms protecting blisters upon the surface to which it is applied. Paraffine wax has a much lower melting point about 120° to 130° Fahrenheit, and it is therefore feasible to apply the wax to the stearin pitch at a temperature considerably above the melting

point of the wax but still well below the melting point of the stearin pitch.

The temperature at which the wax-like material is applied to the flame retarding compound should be well above the melting point of the wax-like material to facilitate its application in a thin film and cause the wax-like material to enter the interstices of the flame-retarding compound, but such temperature of the wax-like material should not be sufficiently high to melt or soften the flame-retarding compound to such a degree that might cause the wax-like material and flame-retarding compound to become mechanically mixed, a condition that would materially decrease the flame-retarding properties of the flame-retarding compound.

To properly correlate the temperatures of the flame-retarding compound and wax-like material for the reasons stated, it is desirable to cool the covered conductor or conduit after the application of the flame-retarding compound and prior to treatment of the wax-like material. To this end the present invention in one of its aspects subjects the covered conductor or conduit to a cooling operation following the application of the flame-retarding compound, and as shown in the present instance of the invention the covered conductor or conduit upon leaving the tank containing the flame-retarding compound is passed about a roll 34 immersed or partially so in a bath of powdered mica, and is then carried an appropriate number of times about the spaced rolls 35 and 36, the latter being preferably, though not necessarily supported in a bath of cooling liquid, and upon reaching the desired cooled condition the covered conductor or conduit may be wound upon a reel 38 preparatory to treatment by the wax-like material.

The flame-proofed covered conductor or conduit is now ready for the wax treatment which may be effected by drawing it from the reel 39 (Fig. 6) into the heated tank 40 containing wax-like material, such for example as paraffin, ceresin, beeswax, ozokerite, Montan wax, carnauba, etc. The wax-like material 41 is applied to the flame-retarding coating 31 in a melted condition but at a temperature that is sufficiently below the melting point of the coating material 31 to prevent the wax material from melting said coating or mixing mechanically to any substantial extent with the flame-repellent coating.

As stated, a primary feature of the invention resides in a covered conductor or conduit having wax-like material applied to the sticky flame-repellent compound to impart to the coating a smooth, clean, non-sticky outer surface, without impairing the flame-repellent properties of the coating. The manner in which the wax-like material is applied to the flame-repellent coating is

important for unless the inflammable wax or paraffin is properly applied so that it does not mix to any substantial extent with the flame-repellent compound it will seriously impair the flame-retarding properties of the coating 31.

As the covered conductor or conduit leaves the tank 40 containing the wax-like material 41, all excess wax material should be removed so that only a film remains, and while various means might be employed to remove the excess wax material, one good construction consists of a die 42 through which the covered conductor or conduit is drawn. This die is made of metal or other hard material and is provided with a bore having the same size or practically the same size as the bore of the die 32. The object in giving both dies 32 and 42 the same size is to cause the latter to iron or force the wax into the interstices of the coating of flame-retarding material without at the same time causing a mixture of the two materials. The die 42 is kept hot by the wax carried upwardly by the covered conductor or conduit and this increases its ironing action so that it irons the surface of the flame-retarding coating to increase its smoothness and at the same time forces the wax into the interstices of the coating to impart to the covered conductor or conduit 14 a smooth, polished surface or "slick finish" that is not sticky.

This wax treatment improves the outer surface of the covered conductor or conduit in many respects without appreciably effecting the flame retarding properties of the coating 31. As a result of this treatment the covered conductor or conduit is rendered non-sticky so that adjacent coils when wound into a package and bound tightly will not stick together even in hot weather, and the powdered mica applied to the cable covering will not flake off since the particles of mica that remain upon the covering when it reaches the die 42 are completely embedded in the cable coating by the pressure of the die. The wax also prevents the flame-retarding coating from oxidizing and adds to the moisture proofing properties of the covered conductor; it also forms a clean, smooth lubricant upon its outer surface that facilitates drawing the cable through conduits and openings during installation.

In order more clearly to indicate in the drawings the successive treatments to which the covered conductor or conduit is subjected, the upper portion of the cable covering 14 of Fig. 1 is shown as untreated, while a portion near the upper end thereof is shown as treated only with the moisture proofing material 21. The lower half of the cable is shown as provided with the flame-retarding coating 31 over a portion of which is applied the wax-like material 41. The

coatings upon the conduit of Fig. 3 are similarly shown.

After the treated covered conductor or conduit leaves the die 42 of Fig. 6 it is passed over a guide roll 43 and is then wound on the take-up reel 44, from which it may be drawn off and wound into coils 45 of the desired length, as shown in Fig. 7, ready for the market, each coiled cable being packed in a box container 46.

The novel protecting coating for cables and conduits forming the subject matter of the present invention may be produced at a very low cost and possesses as one of its most important advantages the complete elimination of the tendency of adjacent coils of a fire-proofed cable or conduit to stick together. This tendency of the treated coils to stick together has been a continuous source of trouble as it not only makes the coils hard to unwind, but frequently causes a section of the flame-repellent coating to be torn from one of the coils as they are forced apart. Through the present invention this difficulty is entirely corrected and adjacent coils will no longer stick together even in the hottest weather.

It will be understood from the foregoing that the wax-like film applied over the stearin pitch or other flame-repellent coating does not penetrate deeply into the surface of the coating and does not mechanically mix with it to any substantial extent or otherwise effect its fire-repellent properties, with the result that the stearin pitch maintains its valuable properties of forming protecting blisters about the cable covering when exposed to high temperatures. These blisters provide a free space between the surface of the blisters and the outer jacket formed of textile or other inflammable material to protect the jacket in an effective manner from the action of the flame. When a conductor covering having the "slick finish" of the present invention is subjected to the action of a flame the wax or paraffin may melt and drop off the stearin pitch leaving the latter in a substantially pure state to form the protecting blisters above mentioned.

An extremely important feature of the present invention resides in the fact that when an insulated conductor or conduit is provided with the protecting coating of the present invention a flame will not travel along the same out of the field of combustion. For instance, in installing electrical conductors a torch is frequently employed in soldering the joints, and if the insulation of the ordinary cable becomes ignited from the torch the flame is likely to creep along the insulation until it reaches some inflammable structure of the building, whereupon a serious fire may be started. It is impos-

sible for a flame to creep along the covering of a conductor having the flame-repellent "slick finish" of the present invention.

While stearin pitch is found in practice

- 5 to form an excellent flame-repellent coating, other forms of fatty acid pitches may be used with more or less success, such for example as palm-oil pitch, bone-fat pitch, cottonseed-oil pitch, cotton pitch, corn-oil 10 pitch, packing-house pitch, etc., and the flame-retarding coating may also be made from various combinations of blown, distilled or fluxed asphalts, native bitumens and similar bituminous materials either 15 with or without mineral fillers. Although paraffin wax is the wax-like substance herein specifically described, it will be understood that other waxes some of which are above suggested, may be used with more or less 20 success, as may also mixtures of various waxes or other wax-like substances such as various of the higher chlorinated products of naphthalene.

The terms "jacket or covering for electrical conductors" and "covered conductor or jacket" have been used in the specification and claims to include electrical conductors or cables having a covering of fibrous material laid about the conductor wire or wires to form a protecting jacket, and also to designate fibrous tubes or conduits adapted to have conductor wires inserted in the tubes after the latter are completed. Likewise the term "wax-like material" has 35 been used in the claims to cover the various materials mentioned in the specification as adapted to be applied to the flame-repellent coating to give the latter a non-sticky outer surface. An insulated conductor or conduit 40 formed in accordance with the present invention possesses not only the desired flame retarding and "slick finish" characteristics as hereinbefore described, but it is flexible and can be bent freely without injury to the 45 flame retarding coating or the film of wax or paraffin, a condition that enables the conductor to be bent about obstructions during installation, put up in coils or on reels for shipment and otherwise bent since the 50 flame retarding covering remains pliable and flexible in the finished product.

What is claimed is:—

1. The method of treating a fibrous jacket or covering for electrical conductors, which 55 consists of coating such jacket or covering with a flame-retarding compound, and applying to the flame-retarding compound coating a film of wax-like material at a temperature below the melting point of the flame-retarding compounds.

2. The method of treating a fibrous jacket or covering for electrical conductors to protect the jacket or covering from combustion, which consists in coating the jacket or covering 60 with a fire-repellent compound, and ap-

plying to the surface of the fire-repellent compound a coating of wax-like material at a temperature above the melting point of the wax-like material and below the melting point of the fire repellent compound. 70

3. The method of treating a fibrous jacket or covering for electrical conductors, which consists in coating the jacket or covering with a heated flame-retarding compound, cooling the flame-retarding compound, and applying thereto a covering of wax-like material at a temperature below the melting point of the fire-repellent compound. 75

4. The method of treating a fibrous jacket or covering for electrical conductors, which 80 consists in coating the jacket or covering with a sticky fire-repellent compound, and applying to the sticky surface of the flame-retarding compound a film of wax-like material at a temperature below the melting point of the fire-repellent compound to impart a slick finish to the jacket or covering. 85

5. The method of treating the outer jacket of an electrical conductor to provide the same with a flame-repellent coating having a slick 90 finish, which consists in applying to the jacket a flame-repellent coating of stearin pitch, then applying melted wax-like material to said coating at a temperature below the melting point of the stearin pitch to 95 form upon the stearin pitch coating a film of wax-like material that renders the coating non-sticky while maintaining unimpaired its flame-repellent properties. 100

6. The method of treating the outer fabric jacket of an electrical conductor to protect the same from fire and impart a slick finished surface, which consists in applying to the jacket a flame-repellent compound that forms a flexible coating that completely 105 covers the jacket, then applying a melted wax-like material to the coating at a temperature in excess of the melting point of the wax-like material and well below the melting point of the flame-repellent compound to form upon said coating a smooth 110 non-sticky outer surface while the flame repellent properties of the coating remain unimpaired. 115

7. The method of treating an electrical conduit or tubular fabric formed of fibrous material, which consists in first subjecting the conduit or tubular fabric to a moisture proofing treatment, then applying to the moisture proofed conduit or tubular fabric 120 a coating of flame-retarding compound, and applying to the moisture and flame-proofed conduit or tubular fabric a wax-like material to impart to the conduit or tubular fabric a non-adhesive outer surface while maintaining unimpaired its flame-retarding properties. 125

8. The method of treating a non-metallic jacket or covering for electrical conductors, which consists in coating the jacket or cov- 130

- ering with a flame-repellent material which remains flexible in the final product, and applying to the flame-repellent material a film of wax-like material to impart a slick finish to the jacket or covering while maintaining unimpaired the fire-repellent properties of the fire-repellent material.
9. In the art of electrical insulation, a non-metallic jacket or covering for electric conductors having a fire-repellent flexible coating and a film of wax-like material applied over said coating.
10. In the art of electrical insulation, a fibrous jacket or covering for electrical conductors having a coating of flexible and sticky flame-retarding material, and a film of wax-like material applied to the coating of sticky flame-repellent material.
11. In the art of electrical insulation, a fibrous jacket or covering for electrical conductors having a coating of stearin pitch and a film of wax-like material applied to the surface of the stearin pitch.
12. A jacket for an electrical conductor formed of fibrous material and having a protecting coating of a flexible and sticky flame-retarding compound and a film of
- wax-like material applied over said compound so that it is substantially unmixed with the material of the flame-retarding compound.
13. A non-metallic outer jacket for an electrical conductor formed of interlocked strands and having a coating of flexible and sticky flame-retarding compound and a film of wax-like material over said coating to give a smooth non-sticky outer surface.
14. In the art of electrical insulation, a fibrous jacket or covering for electrical conductors having a coating of flame-retarding fatty acid pitch, and a film of wax-like material on the flame-retarding fatty acid pitch to impart a slick non-adhesive surface while maintaining unimpaired the flame-repellent properties of the fatty acid pitch.
15. In the art of electrical insulation, a non-metallic jacket having a protective coating of a bituminous flame-retarding compound, and a film of wax-like material applied to the surface of the bituminous flame-retarding compound.

In testimony whereof, I have signed my name to this specification.

OTTO A. FREDERICKSON.